

# UNITED STATES PATENT OFFICE.

DONALD MARKLE, OF HAZLETON, PENNSYLVANIA.

## PROCESS OF FORMING FUEL.

1,407,700.

Specification of Letters Patent. Patented Feb. 28, 1922.

No Drawing.

Application filed March 22, 1920. Serial No. 387,702.

To all whom it may concern:

Be it known that I, DONALD MARKLE, a citizen of the United States, residing at Hazleton, in the county of Luzerne and State of Pennsylvania, have invented a new and Improved Process of Forming Fuel, of which the following is a specification.

In the specification of U. S. Letters Patent No. 1,287,382 granted to me December 10, 1918 I have described a process of forming fuel in which anthracite culm is mixed with hard pitch and the volatile elements of the pitch are distilled off whereby there is produced a dense fuel having the essential qualities of anthracite coal. I have now discovered that by substituting coking bituminous coal for the pitch and mixing this with anthracite culm in proper portions and subjecting the mixture to distillation temperature under proper conditions which I have discovered by experiment I can secure substantially the same results as by the employment of pitch according to my former process. In carrying my invention into effect in order to produce a relatively dense fuel without cell structure, which is the object of my improvements, it is necessary that both the anthracite and bituminous elements shall be finely ground and intimately mingled so as to form a uniform mixture in which fine particles of both are in contact throughout the mass. This enables the fine particles of anthracite to be imbedded in and held by the bituminous element as a matrix when the latter is softened in the course of distillation. If on the contrary, the particles of coal are too coarse, not only will the particles of anthracite fail to be held by the softened bituminous coal, because of the less intimate contact between the two, so that the particles of anthracite will tend to break away or scale off from the mass but there will also be a tendency to the formation of cellular structure in the larger particles of the bituminous coal. Again if the two are not mixed with sufficient intimacy and uniformity so that there is an aggregation of anthracite particles in one place and of bituminous particles in another the aggregated anthracite particles will not be imbedded in and held by the bituminous while there will be a tendency to the formation of cellular coke structure in the aggregation of bituminous particles.

Accordingly in carrying my invention into effect I first grind or pulverize anthracite

culm and coking bituminous coal to such a degree of fineness that approximately 95 per cent of the mass will pass through a 20 mesh screen and 85 per cent through a 40 mesh screen. Further, in order to obtain a sufficiently intimate and uniform admixture of the two, I mix them in any usual or convenient manner before grinding and grind or pulverize them together thus obtaining a uniform distribution of the two throughout the mass. In forming the mixture regard must be had to the relative proportions in which the anthracite and bituminous coal are employed. Thus I find that if the mixture contains less than approximately 25 per cent of coking coal the matrix formed will be insufficient to give the desired degree of cohesion and the particles of anthracite will tend to break away or scale off from the mass, while if as much as 45 per cent of coking coal is employed there is a tendency to develop an undesirable cellular structure like coke, I accordingly preferably employ in the mixture a proportion of coking coal between, or not outside of these extremes, say from 30 to 35 per cent of coking coal to from 70 to 65 per cent of anthracite culm which proportions I find in practice give good results.

This mixture having been pulverized and thoroughly mixed as above described is charged in the mass, that is, without being compacted, into a suitable closed retort, such as an ordinary coke oven and heated at such a temperature and for such a time as to drive off the volatile matter from the coking coal. This is done in the manner ordinarily employed in coking bituminous coal.

Preferably I employ a temperature of 700° C., and upward, a somewhat lower temperature will effect the desired result but is not economically desirable on account of the longer time required.

On account of the loose condition of the mass and the small size of the particles employed the gases given off pass freely out of the retort without causing the development of any cell structure and because of the intimate and uniform contact between the particles of the anthracite and coking coal the former become imbedded in the softened mass of the latter as in a matrix. When the volatile matter has been driven off from the coking coal the mass is discharged from the retort and quenched with water to prevent combustion in the air.

The product thus formed is not coke but

is a very hard and relatively dense homogeneous mass of unchanged particles of anthracite held together by the distillation residue of the coking coal as a matrix.

5 This fuel while not particularly adapted for use in metallurgical operations, since it does not burn throughout the mass but only on the surface, has a high calorific value and burns with a smokeless flame. It is thus 10 equally desirable with ordinary anthracite as a fuel for domestic use or for making steam.

Having thus described my invention what I claim as new and desire to secure by Letters Patent is:—

1. The process of producing a homogeneous, non-cellular carbonaceous fuel which consists in forming a mixture of anthracite slack and coking bituminous coal in 20 the proportion of not less than sixty per cent of anthracite and not more than forty per cent of bituminous, grinding the mixed coals together to such fineness that approximately all the mass will pass through a 20 mesh 25 screen and at the same time intimately mix-

ing the components, charging the mixed mass without compacting into a retort and heating it to such temperature as to soften the bituminous particles and drive off their volatile elements.

2. The process of producing a homogeneous non-cellular carbonaceous fuel which consists in forming a mixture of anthracite slack and coking bituminous coal in the proportion of not less than 60 per cent of anthracite and not more than 40 per cent of bituminous, grinding the mixed coals together to such fineness that 85 per cent of the mass will pass through a 40 mesh screen and 95 per cent thereof through a 20 mesh screen, 30 and at the same time intimately mixing the components, charging the mixed mass without compacting into a retort and heating it to such temperature as to soften the bituminous particles and drive off their volatile 35 elements.

In testimony whereof I affix my signature, this 20th day of March 1920.

DONALD MARKLE.